

June 2, 1931.

H. E. DEPUTY

1,807,689

METHOD OF MAKING COMPOSITE PISTONS

Filed Aug. 20, 1928



Fig. 1.



Fig. 3.



Fig. 2.

Inventor  
Horace E. Deputy

By Swan, Frye & Murray.  
Attorneys

## UNITED STATES PATENT OFFICE

HORACE E. DEPUTY, OF DETROIT, MICHIGAN

## METHOD OF MAKING COMPOSITE PISTONS

Application filed August 20, 1928. Serial No. 300,682.

This invention relates to a process of making composite pistons, and has for its principal object the provision of a simple and effective method of making pistons of two or more metals. Preferably, I desire to combine a metal such as aluminum, or aluminum alloy, to secure the advantage of the relatively light weight, high heat conductivity, and adaptability for machining of such a metal, with a metal having a lower co-efficient of expansion than the aluminum, or alloy thereof, such as cast iron, to overcome the usual disadvantage of aluminum pistons resulting from the relatively high co-efficient of expansion of aluminum and its rapid wear when subjected to friction.

Another object of the present invention is the securing of a substantially permanent bond between piston parts formed of different metals.

Other objects and advantages will be apparent from the following description of a preferred manner of embodying my method of making composite pistons, particularly when taken in connection with the accompanying drawings, wherein:

Figure 1 is a vertical sectional view through a piston constructed in accordance with my improved method.

Figure 2 is a cross section taken substantially on the line 2—2 of Figure 1, and

Figure 3 is a detailed view of the sleeve before being bonded to the body portion of the piston.

In these views the reference character 1 designates the head of the piston, and 2 the relatively thick upper portion of the piston wall having the usual grooves 3 therein to receive sealing rings (not shown). The numeral 4 designates an aluminum or aluminum alloy skirt portion of the piston formed integrally with the parts 1 and 2, while 5 designates a sleeve of cast iron, steel or other metal having a relatively low co-efficient of expansion embracing the skirt portion 4. The sleeve or annulus 5 is rigidly united with the aluminum skirt portion of the piston throughout substantially its entire inner surface, and also the end faces of the sleeve 50 abut and are preferably united with shoul-

ders or flanges 7 and 8 integrally formed with the aluminum skirt portion of the piston.

I have found that by preparing a sleeve or annulus 5 of steel, cast iron or other metal having a relatively low co-efficient of expansion and then placing such sleeve into the mold in which the aluminum portion of the piston is subsequently cast, that the aluminum body of the piston may be rigidly united with the sleeve. In the illustrated embodiment, the entire interior surface of the sleeve has been serrated by cutting a coarse screw-thread spirally along substantially the entire inner surface. The aluminum, when in its original molten state, enters fully between the serrations so as to firmly interlock the two metals. It is to be understood, however, that the sleeve 5 may be formed without any serrations, or that serrations or other forms than screw threads may be substituted for those shown.

To further insure a firm and substantially permanent connection between the sleeve 5 and the aluminum skirt portion 4, it is preferred to subject the sleeve to a preliminary acid bath so as to thoroughly cleanse the surface thereof, and then immerse the sleeve in molten zinc or tin so as to deposit on the sleeve in molecular union therewith a thin coating of zinc or tin. When subsequently the aluminum casting is hardening in contact with the sleeve, the coating also molecularly unites with the aluminum to form the bond between the sleeve and piston skirt.

A still further precaution may be exercised in the interest of an exceedingly rigid bonding between the two metal portions of the piston by highly heating the sleeve 5 preliminarily to pouring the molten aluminum into contact with the sleeve. This heating may range from 400° to 1100° Fahrenheit, the temperature raise preferably being as great as may be employed without resulting distortion or burning of the bonding metals. As the two metals cool, the aluminum alloy will dissipate its heat more rapidly than the cast iron, and the contraction accompanying cooling of the sleeve 5 will increase the

tightness with which it embraces the aluminum. Such pre-heating of the sleeve 5 also avoids a too rapid chilling of the aluminum by the cast iron and such tendencies toward imperfections as might result.

5 In putting my invention into practice, I first provide the desired serrations 6 upon the sleeve 5. I then treat the iron sleeve in an acid solution to cleanse same and remove 10 all grease. The sleeve is then immersed in molten zinc or tin until a desired deposit has been secured thereon. The sleeve is then pre-heated to a desired relatively high temperature and properly positioned in the mold. 15 The molten aluminum or aluminum alloy is then flowed into the mold in the manner well known to those skilled in this art. When the casting has set, the composite piston is preferably plunged into cold water to harden 20 the aluminum or alloy. The mold and its core are, of course, shaped and designed so as to give the desired size and contour to the piston, it being understood that pistons of various sizes and shapes are intended to be 25 made in accordance with my improved method.

During the setting of the molten aluminum within the mold the zinc or tin deposit on the sleeve molecularly unites with the aluminum body portion of the piston adjacent the 30 end faces of the sleeve as well as the entire inner periphery of the sleeve, thereby serving to effectively join the different metallic portions of the pistons to each other, and at the 35 same time the shoulders or flanges 7 and 8 integrally formed with the body portion of the piston serve to definitely position the sleeve.

The piston may now be machined as desired. The piston illustrated herein is provided with the usual pair of diametrically opposed wrist pin bearings 9 which are shown as formed integrally with the aluminum body portion. It is to be understood, however, 45 that other means of securing the wrist pin bearings in position may also be used.

What I claim is:

1. The process of making composite pistons consisting of first heating a metallic sleeve to expand same, placing the expanded sleeve in a heated mold, and then flowing molten metal having a higher co-efficient of expansion than the metal of the sleeve into the mold to engage the entire inner periphery 55 of the sleeve.

2. The process of making composite pistons which consists of providing a metallic sleeve, and then providing upon the sleeve a deposit of zinc alloy, then heating the sleeve to expand same, then placing the expanded sleeve in a heated mold, and finally molding the remainder of the piston in engagement with the inner periphery of the sleeve.

In witness whereof I hereunto set my hand.

65 HORACE E. DEPUTY.